

# United States Patent

[19]

Cameron et al.

[11] 3,894,875

[45] July 15, 1975

[54] **SILVER HALIDE EMULSIONS  
CONTAINING YELLOW DYE-FORMING  
COUPLERS EXHIBITING VERY LOW pH  
SENSITIVITY**

[75] Inventors: **Robert G. Cameron**, North Chili;  
**William J. Gass**, Rochester, both of  
N.Y.

[73] Assignee: **Eastman Kodak Company**,  
Rochester, N.Y.

[22] Filed: **Nov. 28, 1973**

[21] Appl. No.: **419,574**

[52] U.S. Cl..... **96/100**; 96/74; 260/562 R

[51] Int. Cl..... **G03c 1/40**

[58] Field of Search..... 96/100, 74

[56] **References Cited**

UNITED STATES PATENTS

|           |         |                    |              |
|-----------|---------|--------------------|--------------|
| 3,265,506 | 8/1966  | Weissberger et al. | ..... 96/100 |
| 3,408,194 | 10/1968 | Loria              | ..... 96/100 |
| 3,647,452 | 3/1972  | Hendess et al.     | ..... 96/100 |

Primary Examiner—J. Travis Brown  
Attorney, Agent, or Firm—J. T. Lewis

[57] **ABSTRACT**

A class of pivalyl aryloxy ketomethylene color-forming coupler compounds exhibit high reactivity with oxidized color developer over a wide range of alkaline pH conditions. Compounds having this unique capability have the structure:



wherein *n* is from about 9 to about 25 and M is a monovalent cation.

**9 Claims, No Drawings**

SILVER HALIDE EMULSIONS CONTAINING  
YELLOW DYE-FORMING COUPLERS  
EXHIBITING VERY LOW pH SENSITIVITY

This invention relates to color-forming coupler compounds having special utility in the field of photography. More particularly, the present invention relates to a special class of ketomethylene yellow dye-forming compounds and to their use in photographic film elements.

Color-forming coupler compounds are essential components in many phases of contemporary color photography. Ordinarily, they react with oxidized aromatic amino color developing agents to yield colored dyes which contribute to the color of the photographic product. The reaction with color developing agents takes place during the "development" of the photographic element, after the element has been imagewise exposed. Color developing processes have heretofore required very carefully controlled conditions of, for example, time, temperature and pH during the various steps of such processes, particularly the step during which the reaction of color-forming coupler(s) with oxidized color developer material(s) takes place; i.e., the so-called "color development" or "development" step.

One reason for carefully controlling the alkalinity or pH of developer solutions during the color development step of conventional color photographic processing is the very sharp drop-off in the color-forming efficiency of the process at relatively lower developer solution pH's. For example, although the Dmax of the yellow dye formed by reaction of a conventional yellow dye-forming coupler with a conventional oxidized aromatic amino color developer in an otherwise standardized test (which test is described in detail in Example I, below) was 3.40 when a photographic element was developed at a pH of 11.5, the Dmax was only 1.89 when the element was developed at a pH of 10.0. Such a sharp drop-off in Dmax (with some variation in the extent of drop-off with decreasing pH from an optimum pH) can be observed almost invariably with color-forming couplers. Unfortunately the optimum pH for color development often varies somewhat, depending upon the particular color developer, color-forming coupler, or combination of couplers, being used. Such variation creates difficulties for those involved in the manufacture of new, commercially acceptable photographic products.

From this it can be appreciated that there is a present need for color-forming couplers which exhibit an insensitivity to pH over at least a large portion of the useful alkaline developer solution pH range. The existence of pH insensitive couplers would provide greater flexibility to the formulator of photographic emulsions, and to the manufacturer of "color" photographic elements.

DESCRIPTION OF THE INVENTION

It has now been discovered that one limited class of 2-equivalent pivalyl aryloxy ketomethylene color-forming couplers has the surprising capability of being practically insensitive to developer solution pH over a fairly wide range (i.e., pH 9 to pH 12 or wider) of developer solution alkalinities.

Compounds having this unusual capability have the structure A:

5

10 (A)



wherein M is hydrogen or a monovalent cation and n is an integer of from about 9 to about 25. The invention is particularly surprising in view of the fact that many pivalyl aryloxy ketomethylene couplers having structures very similar to those of structure A apparently do not exhibit low insensitivity to pH changes.

DETAILED DESCRIPTION OF THE INVENTION

This invention relates to novel coupler compounds and to photographic emulsions and elements in which such compounds are incorporated.

Although the present invention is broadly applicable to the various compounds encompassed by the formula of structure A, set out above, it is generally preferred that M be hydrogen, ammonium or an alkali metal cation such as lithium, sodium or potassium and that n is an average of from about 11 to about 19. It is still further preferred that M is hydrogen and n is about 15. After the color-forming couplers of this invention are incorporated into a photographic emulsion, the particular identity of M is extremely difficult to determine, and is unimportant insofar as the successful practice of this invention is concerned.

The color-forming couplers of this invention are "incorporated" couplers which are present in the photographic element from the time of manufacture of said element through the color development step of the developing process. The couplers can be incorporated into the photographic emulsion during the emulsion manufacturing operation in any of a number of techniques such as, for example, those described in Section XXII, page 110 of Product Licensing Index, Vol. 92, Dec. 1971. Actually, the particular technique of incorporating the present coupler materials into the photographic emulsions has little or no effect upon the successful practice of the present invention. Generally, however, photographic emulsion containing "incorporated" type couplers which can be dissolved in relatively high boiling coupler solvents (often with the aid of auxiliary solvents in the usual manner) are prepared by first dispersing in aqueous gelatin solutions the coupler (dissolved in a solvent comprising a high boiling crystalloidal coupler solvent and an auxiliary organic coupler solvent having substantial solubility), then causing the resulting coupler dispersion in gelatin to set, washing this "set" dispersion to remove a substantial amount of the auxiliary solvent with an aqueous solution (at a pH within about 0.5 units of the isoelectric point of the gelatin) of a carboxylic acid having 2-8 carbon atoms such as propionic acid, and subsequently blending the washed dispersion with a gelatino silver halide emulsion.

Similarly, the other specific components which are present in the photographic emulsions and elements of this invention are not critical with respect to the present invention so long as the emulsions are photosensitive silver halide emulsions. Such emulsions contain hydrophilic colloid such as gelatin and can contain addenda, as desired, such as hardeners, antifoggants, sensitizing dyes, chemical sensitizers, coating aids, plasticizers, coupler solvents, matting agents, brighteners, and the like without distracting excessively from the successful practice of the invention. Many examples of such hydrophilic colloids and addenda, and means for their use can be found in Product Licensing Index, Vol. 92, December 1971, pages 107-110, publication 9232.

The present couplers are "ballasted" in that they remain essentially immovable in the emulsion, after the emulsion is dried. These couplers convert into a yellow dye upon reaction with oxidized color developer. For example, upon reaction with N,N'-diethylamino-p-phenylene diamine, the coupler of Structure A wherein M is hydrogen and n is 15 is converted into a very desirable yellow dye having a peak absorbance at 444.1 nanometers. Because of their yellow dye-producing capability the couplers of this invention are almost invariably incorporated into the so-called "blue sensitive" layer of a 3-color photographic element. Generally, this blue-sensitive layer is the topmost layer of a three layer element (which may contain additional layers over, between and under the three basic color-forming layers, as desired), the remaining color-forming layers being "green-sensitive" and "red-sensitive," in the typical, wellknown fashion.

The photographic emulsions of this invention (which contain the color-forming coupler compounds of Structure A) are generally coated in any desired manner in the form of at least one layer on a photographic support. The particular support that is used is not important with respect to the successful practice of this invention. Typical photographic supports are described and referred to in Product Licensing Index, Vol. 92, Dec. 1971, Section X.

Organic amino aromatic color developing materials are well known in the art and need not be described in detail here. The couplers of the present invention can be "developed" with solutions containing any organic amino aromatic color developing material that is useful for conventionally color developing photographic elements containing incorporated colorforming couplers. Typical, non-limiting examples of such organic amino aromatic color developing materials include p-aminophenol, p-phenylenediamine and N,N-diethyl-p-phenylenediamine. It should also be noted that, manipulatively, conventional color development processes can be used successfully to develop photographic elements containing the present couplers incorporated in at least one of the layers thereof.

#### EXAMPLE

In the following example, all "parts" given are by weight unless otherwise specified.

A. A series of photographic elements were prepared by coating in a conventional manner onto a conventional cellulose acetate film support layers of photographic emulsions, each containing 11.1 mg/sq. decimeter of silver (as iodobromide) and  $2.8 \times 10^{-5}$  moles/sq. decimeter of yellow dye-forming coupler. Each

of the element samples contained a different coupler, identified as Coupler 1 through 13, below. The couplers were incorporated into the emulsion by the method set out in U.S. Pat. No. 2,322,027.

B. Each of the elements manufactured in accordance with part A of this example was cut into four segments, exposed to a conventional graduated density test object, and then developed for 4 minutes using Kodak CD-3 Developer and processed completely in a conventional way. However, prior to the developing step, the pH developer solution was adjusted by conventional means to pH's of 10.1; 10.5; 11.0; and 11.5. In Table I, below, are set out the values for Dmax of each of the elements prepared as in paragraph A of this example.

Kodak CD-3 Developer is a solution of 4.5 g sodium sulfite, 36 g anhydrous potassium carbonate, 0.75 g potassium bromide, 0.09 g potassium iodide, 1.0 g diethaoctanediol, 0.1 g tetramethyl ammonium hydrotriborate, and 7.0 g 4-amino-3-methyl-N-ethyl- $\beta$ -(methanesulfonamido)ethylaniline sesquisulfate in water, made to 1 liter.

Table I

| Coupler No. | 10.0 | Dmax at pH* |      |      |
|-------------|------|-------------|------|------|
|             |      | 10.5        | 11.0 | 11.5 |
| 1           | 3.10 | 3.10        | 3.08 | 3.08 |
| 2           | 2.36 | 3.18        | 3.46 | 3.43 |
| 3           | 2.33 | 3.20        | 3.48 | 3.44 |
| 4           | 2.60 | 3.16        | 3.68 | 3.30 |
| 5           | 2.80 | 3.08        | 3.62 | 3.20 |
| 6           | 2.56 | 3.18        | 3.34 | 3.48 |
| 7           | 3.14 | 3.70        | 3.72 | 3.80 |
| 8           | 1.89 | 2.68        | 3.23 | 3.40 |
| 9           | 1.34 | 2.50        | 3.06 | 3.32 |
| 10          | 2.62 | 3.43        | 3.37 | 3.17 |
| 11          | 2.83 | 3.20        | 3.24 | 3.05 |
| 12          | 2.66 | 3.21        | 3.34 | 3.06 |
| 13          | 1.96 | 2.38        | 2.98 | 3.25 |
| 14          | 3.36 | 3.56        | 3.32 | 3.70 |

\*pH of developer solution

From the data in Table I, it can readily be appreciated that only coupler number 1 shows consistent non-sensitivity to variations in the pH of developer solutions through the developer solution pH range of from 10 to 11.5, while coupler No. 14 demonstrates only a slight tendency to "lose" Dmax with decreasing developer alkalinity. The couplers used in this test are identified below. While this test was made using only one color developer solution, it is believed that similar comparative results would be obtained using other color developer solutions.



$\alpha$ -Pivalyl- $\alpha$ -(p-carboxyphenoxy)-2-chloro-5-(n-hexadecanesulfonamido)acetanilide



Coupler No. 6



7

Coupler No. 8



8

Coupler No. 9



Coupler No. 10



Coupler No. 12



Coupler No. 11



Coupler No. 13



## Coupler No. 14



scribed in U.S. Pat. No. 3,265,506 and 3,408,194 for example.

The invention has been described in detail with particular reference to preferred embodiments thereof, but, it will be understood that variations and modifications can be effected within the spirit and scope of the invention.

What is claimed is:

1. A light-sensitive silver halide emulsion containing a color-forming coupler compound capable of high reactivity over a wide alkaline pH range; said coupler having the structure:



From the foregoing example, it can be appreciated that the coupler compounds of the present invention exhibit unique properties, as compared with coupler compounds having very similar structures. The reason for this apparently unique capability is not presently known.

The coupler compounds of the present invention also exhibit a surprising capability with respect to their reactivity with oxidized color developing materials in the presence of competing couplers such as, for example, citrazinic acid. For some reason, the present compounds exhibit a continued, high reactivity toward oxidized color developer even in the presence of competing couplers, so that competing couplers appear to

wherein  $n$  is an integer from about 9 to about 25 and M is hydrogen or a monovalent cation.

2. A light-sensitive silver halide emulsion as in claim 1, wherein  $n$  is from about 11 to about 19.

3. A light-sensitive silver halide emulsion as in claim 1, wherein  $n$  is about 15.

4. A light-sensitive silver halide emulsion as in claim 1, wherein  $n$  is about 11.

5. A photographic element comprising a photographic support coated with at least one photosensitive silver halide emulsion layer; said layer containing light-sensitive silver halide, hydrophilic colloid, and a color-forming coupler having the structure:



have relatively little effect on the yellow dye Dmax that can be formed in photographic elements in which the present coupler compounds are incorporated. This particular capability of the coupler compounds of this invention (and some other yellow dye-forming coupler compounds) is detailed at greater length in copending U.S. Pat. application Ser. No. 419,573, filed concurrently herewith, now abandoned, and entitled "Photographic Elements Containing Color-Forming Couplers Having An Inhibiting Effect Upon the Reactivity of Competing Couplers".

The color coupler compounds of this invention can be made by well-known procedures such as those de-

55 wherein  $n$  is an integer from about 9 to about 25 and M is hydrogen or a monovalent cation.

60 6. A photographic element as in claim 5, wherein said color-forming coupler is present in said layer in an amount equal to about  $3 \times 10^{-5}$  moles per square decimeter.

65 7. A photographic element as in claim 6, wherein said n is from about 11 to about 19.

8. A photographic element as in claim 6, wherein said n is about 15.

9. A light-sensitive silver halide emulsion as in claim 6, wherein n is about 11.

\* \* \* \* \*